

H. BURGESS.

Process for Coating Iron with Copper or Brass.

No. 11,319.

Patented July 18, 1854.



# UNITED STATES PATENT OFFICE.

HUGH BURGESS, OF KENTISH TOWN, COUNTY OF MIDDLESEX, ENGLAND.

## METHOD OF COATING IRON WITH BRASS OR COPPER.

Specification forming part of Letters Patent No. 11,319, dated July 18, 1854.

*To all whom it may concern:*

Be it known that I, HUGH BURGESS, of No. 27 Grove Terrace, Kentish Town, in the county of Middlesex, England, have invented or discovered a new and useful Process for Coating Iron with Copper or Brass; and I do hereby declare the following to be a full, clear, and exact description of the manner of doing the same.

This invention consists of cleansing sheets, bars, and other forms of iron to be first cleansed, then coated over with a solution of cadmium or zinc, then dried and dipped into a bath of melted copper or brass, then raised out of the bath into an atmosphere of steam and carbonic acid flowing in jets; and, when the form of the iron will admit of it, a pair of rollers is the best mode of raising out of the bath and equalizing the surfaces; and the reheated sheets or bars may be further rolled, and by like means two surfaces of iron may be coated and joined; and in order that my invention may be most fully understood and readily carried into effect, I will proceed to describe the means pursued by me.

In order that all parts of any article of iron may be well and completely coated with copper or brass by this process, care must be taken in the selection of the iron from which the article to be coated is made, since from the use of dirty scrap-iron, of which much bar and bolt iron is formed, imperfect welding of the parts results; and when the mass of forged iron is rolled into bar or bolt iron the imperfect welding is shown by longitudinal cracks and flaws down the rod or bar, which are not only impossible to clean so as to prepare the bar for the process hereinafter described, but on being suddenly heated by being immersed in the molten copper or brass the flaws open and the dirty surface of the iron prevents the coating being effected in such parts.

I will now proceed to describe the process by which a coating of copper or alloys of copper is effected.

The articles to be coated are to be first well cleaned in dilute sulphuric acid, as is well understood. They are then to be carefully washed in a dilute solution of chloride of zinc. The strength of the solution I have used is made by adding about five parts of water to a saturated solution of the chloride, formed by

dissolving zinc in hydrochloric acid till action has ceased.

I may here state that I do not confine myself to the use of chloride of zinc. I find the other soluble salts of zinc and tin may be used, and oxide of zinc deposited on the article to be coated by holding it in the fumes of zinc during combustion. Oxides of zinc made into a very thin cream with water and applied to the iron article, carbonates of zinc treated in the same way, are all applicable for the process herein described; or in place of zinc cadmium may be used in like manner.

The articles, after having been well dried, when any of the above solutions have been used, may be heated to about 250°, or to any temperature short of driving off or decomposing any of the above-named preparations, and may be plunged into melted copper or alloy of copper.

I may state that I do not find it advisable to use pure copper alone, but that a mixture of about two per cent. of zinc and one per cent. of tin to ninety-seven parts of copper answer the purpose better than copper alone.

The length of time which the article should remain in the molten metal depends on the bulk of the articles and the temperature of the molten metal, and can only be determined by the eye and experience. A three-quarter-inch bolt requires about three seconds. The upper surface of the molten metal should be the hottest, and I have found it desirable to cover the top of the metal with powdered charcoal, sand, or some such substance, to prevent oxidation and the chilling effect of the air. Immediately upon the article being taken out of the metal it is at once introduced into a reservoir or tank containing an atmosphere of steam and carbonic acid flowing into it in streams or in place thereof it may be of carbureted hydrogen or any deoxidizing vapor, and there allowed to cool. Should carbureted hydrogen be used, care must be taken that no atmospheric air be admitted into the reservoir, and for this purpose the entrance by which the coated articles are introduced must be double-valved and the gas kept to a slight pressure, so that the pressure of the gas outward will prevent the introduction of atmospheric air into the tank or vessel, and the double valve will prevent the loss of much gas,

the articles being introduced between the valves, one being shut when the other is open. The tanks should be in sets of two, so that all the gas may be withdrawn from one and passed into the other when it is requisite to remove the coated articles. It is advisable to cover the floors of the tanks with fine sand, to prevent the articles being injured in passing into the reservoir.

The advantage of using carbureted hydrogen or other deoxidizing agents is that the heat from the melting-furnace is quite sufficient to produce all the carbureted hydrogen required, a small retort to distill the coal being placed in the fire of the furnace.

In some instances it may be desirable to protect the coated articles from oxidation by drawing them through a covering of flux on the surface of the molten metal. I effect this by drawing the flux on one side by a fire-clay scraper, immersing the article in the copper, and then allowing the flux to again cover the surface of the metal and withdrawing the article through the flux. I have found that glass answers the purpose well. Iron being lighter than copper or the alloys of copper, I take advantage of this circumstance, and by loosely placing a bolt which is to be coated in an instrument consisting of two cones or rings (at a distance apart according to the length of bolt) that receive the head and point, and which allow it to play, the bolt will rise and fall as it is introduced or withdrawn from the molten metal, and thus all parts are exposed to the hot metal. The cones are made of fire-clay or iron coated with a mixture of some fire-clay and a little borax, and are made as open as is consistent with sufficient strength. The lower cone is attached to a rod of iron protected as the cones, and standing out a little from it. The upper cone is attached to a slide, which is retained at any height on the rod by a screw, the two cones being opposite and one above the other. A bolt is placed with the head in the lower cone, and the upper one is brought down so as to just take in the point, allowing it to rise about an inch and a half, but not sufficient to allow the head to rise out of the lower cone. On being introduced into the molten metal when at a certain depth, the bolt rises and allows the metal to touch all parts of the head. The reverse takes place on withdrawing the bolt. More than one set of cones may be attached to a rod.

For coating small articles I have found a pot with its mouth built into the furnace-mouth, like a glass pot, do very well. The principal object is to keep cold air from the surface of the metal, which must be the hottest part, and to exclude all dust and dirt from the metal. For large processes an air or reverberatory furnace is preferable.

In order to give to the coated iron bolts points of mixed metal, the coated bolts are treated in the following manner: I find a mixture of two per cent. of tin and one per cent. of zinc best for this purpose. The bolts after

having been coated with copper or brass have their end or ends brought up to a blunt point, cleaned, or brightened. They are then fitted into a casting-box, having a bottom perforated with holes. Each hole has a screw attached to it, so that the bolts may be held in the holes by the screws at any desired height. The casting-box is provided with an outlet, the bolts being placed in the box at the desired height. About two inches of loam is sifted over the bottom of the box, the bolts standing out of the loam and showing a little of the coating above the loam. About one-eighth of an inch is sufficient. Runners are then made in the loam from each point and all terminate in the outlet of the box before named. The upper casting-box being of the height of the desired metal points or ends, is placed on the other, as is done in brass-casting. A thin piece of pipe is slipped over the iron end of the bolts, the thickness of the pipe determining the size of the intended point. The point should be about one-sixteenth of an inch larger than the size of the bolt and rolled down to the same diameter. The upper box is now filled up with loam, as is well understood by brass-founders.

I have found it desirable to have a flat top with holes exactly the size of the pieces of pipe which form the pattern for the metal joints, and directly above the holes through which the bolts are placed at the bottom of the box, fitted on the top of the upper box, so as to prevent the patterns being displaced by the ramming. The patterns are withdrawn and runners made from one main to all the molds. The bright iron points are now moistened with any of the above-mentioned solutions or matters and dried by placing a coke-fire over them in an iron basket. The molten copper or alloy of copper may be run from an air-furnace. Sufficient metal must be allowed to flow upon the iron points till they are red hot. The aperture or outlet of the lower box may now be closed with a plug of loam and the points allowed to cool.

I also propose casting copper or brass around iron-bar, bolt, or sheet—and rolling the combined metals when at the requisite temperature. In carrying out this process I proceed as follows: The iron to be coated must be cleaned and washed or covered with any of the substances before mentioned. A mold is prepared of well-dried loam, the same as is used for cores by brass-founders, having a foot at the lower end for the iron to fit into to keep it in its place. An iron bar formed to receive the upper end of the iron serves the same purpose. At the top a small runner is left from the bottom of the mold. The iron being dipped into the metal it is desired to cover it with, it is plunged at once into the mold, which is at the same time filled with molten metal. A little metal is allowed to flow through the lower runner. It is then closed and the mold and feeder filled up with molten metal. A small but strong jet of coal-gas may be made to play upon the iron as it

descends into the molten metal in the mold, the form of the jet being circular, and is brought into close contact with the coated iron by means of a hollow ring, the aperture being just the size of the coated iron, the gas entering the collar by a series of holes in the outside edge of the collar. The combined metals should be rolled as soon as they are cooled to the proper temperature. This varies with the alloy of copper used. In rolling headed bolts I use rollers having a groove in each the size of half the bolt head and shank, so that when the corresponding grooves in the two rollers come together they are equal in size to the head and shank of the bolt. The bolts are placed head first between the rollers.

The accompanying drawings represent the most important of the mechanical appliances used in reducing this process to practice, in which said drawings Figure 1 represents a side view of a molding-box. Fig. 2 represents a top view of the lower part of the molding-box when separated at the red line  $x\ x$  of Fig. 1. Fig. 3 represents a vertical cross-section through the molding-box at the red line  $y\ y$  of Fig. 1. Fig. 4 represents a side view of the gas-box. Fig. 5 represents a vertical central section through the same, and Fig. 6 represents the dipping apparatus.

Similar letters where they occur refer to like parts.

In Figs. 1, 3, A represents the upper, and B the lower, part of the casting-box, held together in any of the usual well-known ways, the latter figure representing the box as filled with sand, and having a bolt,  $a$ , in place to receive a copper or brass point. The ends of the bolts to be coppered are brought to a point, which point protrudes a little above the sand in the lower part, B, of the casting-box. F represents a molding-stick of about the diameter of the bolts, which are placed over the points of the bolts, and should be kept in their true position by guides on top of the casting-box. Sand is then sifted into the upper box and rammed as in the usual way. The molding-sticks are then withdrawn and a pattern of the future copper point is formed. The molding-stick may be a piece of a tube of the diameter or a little larger than the bolt, placed on a piece of wood of the same diameter, the tube being for the purpose of allowing the point of the bolt to enter it, as seen in Fig. 3, and may,

of course, be arranged in sets to suit the number of holes in the casting-box.

In Fig. 2, G represents the holes through which the points of the bolts to be coppered protrude, and  $a'$  is a runner through the center of that part of the casting-box, and which leads to the spout E, and into which runner  $a'$  small runners  $b$  from the bolt-points are brought. The melted metal is run into the pattern d, Fig. 3, passes through the runner  $a'$  and branches  $b$  around the points of the bolts, and runs off at the spout E into any proper vessel to receive it. As soon as the points become red-hot the spout is plugged up and the pattern d filled up and the whole allowed to cool.

Figs. 4, 5 represent the gas-chamber, in which  $e$  represents the upper door, and  $f$  the lower one, both being held shut by springs  $g\ h$ , and the inner door is also provided with a rod or thumb-piece,  $i$ , extending outside, so that it may be opened from the outside. The purpose of this gas-chamber is fully described in the detail of the process.

Fig. 6 represents the dipping apparatus, on which one of the arms H should be made adjustable to receive bolts of variable lengths, and said arm instead of being straight may be curved or inclined, but in such manner that its fingers  $k$  may be directly over the fingers  $l$  of the lower arm, I.

Having thus fully described the nature of my invention or discovery, I desire to state that I do not claim any of the apparatus or the process to which they refer, having described them for the purpose of explanation only; but

What I do claim herein as new, and desire to secure by Letters Patent, is—

The coating of iron sheets, bars, bolts, and other forms of iron with copper or brass by a combination of processes as follows: by first cleaning, then coating them over with a solution of cadmium or zinc, drying and dipping them into a bath of melted copper or brass, and raising them out of the bath into an atmosphere of steam and carbonic acid flowing in streams or in jets, substantially in the manner described.

HUGH BURGESS.

Witnesses:

A. B. STOUGHTON,  
SAM'L. GRUBB.